

111

## UNITED STATES PATENT OFFICE.

JOSEPH FRANCIS KING, OF PHILADELPHIA, PENNSYLVANIA, ASSIGNOR OF ONE-HALF  
TO HARRY B. HAINES, OF PHILADELPHIA, PENNSYLVANIA.

## PROCESS OF BLEACHING.

1,321,644.

Specification of Letters Patent. Patented Nov. 11, 1919.

No Drawing.

Application filed June 28, 1919. Serial No. 307,266.

*To all whom it may concern:*

Be it known that I, JOSEPH FRANCIS KING, a citizen of the United States, and a resident of the city of Philadelphia, county 5 of Philadelphia, and State of Pennsylvania, have invented certain new and useful Improvements in Processes of Bleaching, of which the following is a specification.

My invention relates to a process of 10 bleaching materials, such as cotton, linen, and other plant fibers, textile goods and similar materials as well as wool, silk, and other animal fibers.

An object of my invention is to produce 15 bleached goods of superior quality by a new and useful process of bleaching.

Other objects are to produce a stronger bleached goods; to save time and labor, to reduce the loss in weight of the bleached 20 goods and to improve the appearance of such goods.

Another object of my invention is to bleach such materials when desired to a "dead white" as contra-distinguished from 25 bleaching effects known as "half-bleach".

Another object is to remove, during the bleaching operation, the foreign matter, such as specks, motes and shives, found for example, in raw cotton, and which, when 30 present in bleached materials, affects the value and appearance thereof.

In prior bleaching processes within my knowledge, several disadvantages are present, among which are the great length of 35 time necessary to complete the bleaching action, the large amount of labor involved, the large number of handlings and treatments necessary, the loss in weight and tensile strength of the bleached material, the 40 failure to obtain a bleached product with a high grade of softness or "loft" and the presence of foreign matter or impurities.

By the process of my invention all of the 45 above disadvantages are sought to be overcome or remedied and in carrying out my invention I find that a complete bleaching action may be accomplished in approximately two hours with a large saving in labor involved, and with the number of 50 handlings and treatments of the material to be bleached reduced to a minimum. I also find that by my process there is often-times no loss in weight of the bleached material and whenever such loss occurs it 55 rarely exceeds two per cent. I further find

that by my process the loss in tensile strength of the bleached material is substantially decreased and also that the bleached material is of a superior grade both in quality and appearance, its loftiness being 60 markedly superior to that obtained in the chlorid of lime process of bleaching.

Moreover, by my process, impurities, such as specks, motes, shives and the like which detract from the appearance and the value 65 of the material or goods, are eliminated, with the result that the appearance of the material is greatly improved and the value thereof enhanced.

In carrying out my invention I first prepare a bleaching compound or composition by mixing together the following enumerated constituents or ingredients in substantially the proportions indicated as follows:

10 parts by weight of common salt or sodium chlorid,

10 parts by weight of soda ash or sodium carbonate,

6 parts by weight of peroxid of hydrogen,

10 parts by weight of caustic soda or potassium hydrate,

24 parts by weight of Glauber salt or sodium sulfate.

I may then place 500 gallons of water in a suitable vat to and in which I may add 85 and dissolve 60 pounds of the above bleaching composition or mixture and then place in said solution 1000 pounds of material to be bleached.

The contents of the vat then may be boiled 90 for approximately an hour after which the materials are rinsed, first in hot water for about five minutes and then in cold water for also about five minutes.

If, however, it is desired to dye the materials, any particular color, the bleaching process may be carried out with about substantially one-half of the quantity of the bleaching composition or mixture mentioned above and for about one-half of the time 100 necessary for a complete bleaching.

The dye may be first prepared by forming a dye paste by mixing, as for example, "sky-blue" dye with a little warm water and then dissolving four ounces of this in two gallons 105 of cold water. This dye solution may then be added to the cold water rinse and the goods in the vat and allowed to stand for about five minutes. The contents of the vat may then be heated to about 130° Fahren- 110

heit and left for about five minutes to produce a light shade of dyeing or for such longer periods as may be required to produce deeper shades. By this method substantially any desired shade may be obtained.

In the process described above, the function of the caustic soda in conjunction with the sodium carbonate is primarily for the purpose of cleansing the material of impurities, while the remaining constituents primarily react to cause the bleaching action.

If, then, the materials are already free of impurities it may not be necessary to give them the particular treatment required to remove such impurities and my process may omit the constituents sodium carbonate and caustic soda. From the above it may be observed that this solution is alkaline but depending upon the materials to be treated acids may be substituted for alkalis as desired.

In addition to the above operation, I find, if desired, that I can use reels and squeeze rolls for the goods when bleaching and rinsing the same.

While I have above described the manner in which materials may be bleached, this description is intended as exemplifying rather than limiting my invention and it is to be understood that the materials used, their proportions, the order in which the steps are enumerated and the period of treatment, may be suitably varied without departing from the spirit and scope of my invention.

Having thus described my invention, I claim and desire to protect by Letters Patent of the United States:

1. The process of bleaching consisting of

dissolving sodium chlorid, sodium carbonate, hydrogen peroxid, potassium hydrate and sodium sulfate in water, introducing the materials to be bleached into said solution, subjecting the mass to heat and rinsing the bleached materials.

2. The process of bleaching consisting of placing the material to be bleached in a bleaching solution containing sodium chlorid, sodium sulfate and hydrogen peroxid and boiling said material and solution.

3. The process of bleaching consisting of placing the material to be bleached in a bleaching solution containing sodium chlorid, sodium sulfate and hydrogen peroxid, boiling said material and solution and rinsing said bleached material.

4. The process of bleaching and coloring consisting of dissolving a mixture of sodium chlorid, sodium carbonate, potassium hydrate, sodium sulfate and hydrogen peroxid in water, placing the material to be bleached and colored in said solution, heating said material and solution, rinsing said material with water, applying a soluble coloring substance to the rinsing water containing the bleached material and heating said material and colored solution.

5. The process of bleaching consisting of dissolving a mixture of common salt, Glauber salt, hydrogen peroxid and a detergent in water; placing the material to be bleached in said solution, boiling said solution and material and washing said bleached material.

In witness whereof I have hereunto set my hand this 27th day of June, 1919.

JOSEPH FRANCIS KING.